

## [54] THIAZOLYLMETHYLENE-2-PYRAZOLINE-5-ONE DYE-DONOR ELEMENT FOR THERMAL DYE TRANSFER

[75] Inventors: Steven Evans, Rochester; Helmut Weber, Webster, both of N.Y.

[73] Assignee: Eastman Kodak Company, Rochester, N.Y.

[21] Appl. No.: 290,604

[22] Filed: Dec. 23, 1988

[51] Int. Cl. 4 ..... B41M 5/035; B41M 5/26

[52] U.S. Cl. ..... 503/227; 8/471; 428/195; 428/480; 428/913; 428/914

[58] Field of Search ..... 8/471; 428/913, 914; 428/195, 480; 503/227

## [56] References Cited

## U.S. PATENT DOCUMENTS

|           |         |                |               |
|-----------|---------|----------------|---------------|
| 4,701,439 | 10/1987 | Weaver et al.  | ..... 503/227 |
| 4,743,582 | 5/1988  | Evans et al.   | ..... 503/227 |
| 4,760,049 | 7/1988  | Etzbach et al. | ..... 503/227 |

## FOREIGN PATENT DOCUMENTS

239290 11/1985 Japan ..... 503/227

Primary Examiner—Bruce H. Hess

Attorney, Agent, or Firm—Harold E. Cole

## [57] ABSTRACT

A dye-donor element for thermal dye transfer comprises a support having thereon a dye dispersed in a polymeric binder, the dye comprising a thiazolylmethylene-2-pyrazoline-5-one. In a preferred embodiment, the dye has the formula:



wherein R<sup>1</sup> represents hydrogen, a substituted or unsubstituted alkyl group having from 1 to about 10 carbon atoms, a cycloalkyl group having from about 5 to about 7 carbon atoms, or a substituted or unsubstituted aryl or hetaryl group having from about 2 to about 10 carbon atoms;

R<sup>2</sup> represents an alkoxy group having from 1 to about 10 carbon atoms or a primary, secondary or tertiary amino group;

R<sup>3</sup> and R<sup>4</sup> each represents R<sup>1</sup>, with the proviso that only one of R<sup>3</sup> and R<sup>4</sup> may be hydrogen, or R<sup>3</sup> and R<sup>4</sup> can be joined together to form, along with the nitrogen to which they are attached, a 5- or 6-membered heterocyclic ring;

R<sup>5</sup> and R<sup>6</sup> each independently represents hydrogen; halogen; cyano; thiocyanato; a substituted or unsubstituted alkyl, alkoxy, alkylthio or alkylsulfonyl group having from 1 to about 10 carbon atoms; a substituted or unsubstituted aryl or hetaryl, aryloxy or hetaryloxy, arylthio or hetarylthio, arylsulfonyl or hetaryl sulfonyl group having from about 2 to about 10 carbon atoms; a cycloalkyl group having from about 5 to about 7 carbon atoms; alkoxycarbonyl; aryloxycarbonyl; acyl; carbamoyl; mono- or dialkylamino; mono- or diarylamino acylamido; sulfonamido; or sulfamoyl.

20 Claims, No Drawings

THIAZOLYLMETHYLENE-2-PYRAZOLINE-  
5-ONE DYE-DONOR ELEMENT FOR THERMAL  
DYE TRANSFER

This invention relates to dye-donor elements used in thermal dye transfer which have good hue and dye stability.

In recent years, thermal transfer systems have been developed to obtain prints from pictures which have been generated electronically from a color video camera. According to one way of obtaining such prints, an electronic picture is first subjected to color separation by color filters. The respective color-separated images are then converted into electrical signals. These signals are then operated on to produce cyan, magenta and yellow electrical signals. These signals are then transmitted to a thermal printer. To obtain the print, a cyan, magenta or yellow dye-donor element is placed face-to-face with a dye-receiving element. The two are then inserted between a thermal printing head and a platen roller. A line-type thermal printing head is used to apply heat from the back of the dye-donor sheet. The thermal printing head has many heating elements and is heated sequentially in response to the cyan, magenta and yellow signals. The process is then repeated for the other two colors. A color hard copy is thus obtained which corresponds to the original picture viewed on a screen. Further details of this process and an apparatus for carrying it out are contained in U.S. Pat. No. 4,621,271 by Brownstein entitled "Apparatus and Method For Controlling A Thermal Printer Apparatus," issued Nov. 4, 1986, the disclosure of which is hereby incorporated by reference.

A problem has existed with the use of certain dyes in dye-donor elements for thermal dye transfer printing. Many of the dyes proposed for use do not have adequate stability to light. Others do not have good hue. It would be desirable to provide dyes which have good light stability and have improved hues.

JP 60/239,290 and U.S. Pat. No. 4,701,439 relate to arylidene dyes used in a thermal transfer sheet. All of these dyes, however, are benzylidenemalononitriles and do not contain thiazolylmethylene or 2-pyrazoline-5-one structural fragments. In addition, these dyes have poor light stability as will be shown hereinafter.

U.S. Pat. No. 4,760,049 relates to thiazolylmethylenetype arylidene dyes for use in a thermal transfer sheet. However, none of these dyes contains the 2-pyrazoline-5-one fragment. In addition, these dyes have poor light stability as will be shown hereinafter. It would be desirable to provide thiazolylmethylenetype arylidene dyes which have improved hues and stability to heat and light.

Application Ser. Nos. 168,838 entitled "Alpha-cyano Arylidene Pyrazolone Magenta Dye-donor Element For Thermal Dye Transfer" and 168,840 entitled "Arylidene Pyrazolone Dye-Donor Element for Thermal Dye Transfer" by Evans et al. filed Mar. 16, 1988, relate to phenylmethylen-type dyes having a 2-pyrazoline-5-one fragment, but do not have the thiazolylmethylen fragment of the dyes described herein.

Substantial improvements in light stability and hues are achieved in accordance with this invention which comprises a dye-donor element for thermal dye transfer comprising a support having thereon a dye dispersed in a polymeric binder, the dye comprising a thiazolyl-

methylene-2-pyrazoline-5-one. In a preferred embodiment, the dye has the formula



wherein R<sup>1</sup> represents hydrogen; a substituted or unsubstituted alkyl group having from 1 to about 10 carbon atoms, such as methyl, ethyl, propyl, isopropyl, butyl, pentyl, hexyl, methoxyethyl, benzyl, 2-methanesulfonamidoethyl, 2-hydroxyethyl, 2-cyanoethyl, methoxycarbonylmethyl, etc.; a cycloalkyl group having from about 5 to about 7 carbon atoms, such as cyclohexyl, cyclopentyl, etc.; or a substituted or unsubstituted aryl or hetaryl group having from about 2 to about 10 carbon atoms, such as phenyl, pyridyl, naphthyl, thienyl, pyrazolyl, p-tolyl, p-chlorophenyl, or m-(N-methyl sulfamoyl)phenyl;

R<sup>2</sup> represents an alkoxy group having from 1 to about 10 carbon atoms, such as methoxy, ethoxy, 2-methoxyethoxy, chloroethoxy, benzyloxy, phenoxy, isopropoxy, n-butoxy, or n-hexoxy; or a primary, secondary or tertiary amino group, such as amino, N-methylamino, N-ethylamino, N-butylamino, N,N-dimethylamino, N,N-diethylamino, N-methyl-N-propylamino, anilino, morpholino, N-ethylanilino, 2-methoxyethylamino, 2-thienylamino, etc.;

R<sup>3</sup> and R<sup>4</sup> each represents R<sup>1</sup>, with the proviso that only one of R<sup>3</sup> and R<sup>4</sup> may be hydrogen, or R<sup>3</sup> and R<sup>4</sup> can be joined together to form, along with the nitrogen to which they are attached, a 5- or 6-membered heterocyclic ring such as pyrrolidine, morpholine, piperidine, imidazolidine, pyrazole, pyrazolidine, pyrrole, indole, etc.; and

R<sup>5</sup> and R<sup>6</sup> each independently represents hydrogen; halogen, such as chlorine, bromine, or fluorine; cyano; thiocyanato; a substituted or unsubstituted alkyl, alkoxy, alkylthio or alkylsulfonyl group having from 1 to about 10 carbon atoms such as methyl, ethyl, propyl, isopropyl, butyl, pentyl, hexyl, methoxyethyl, benzyl, methylthio, butylthio, benzylthio, methanesulfonyl, pentanesulfonyl, methoxy, ethoxy, 2-methanesulfonamidoethyl, 2-hydroxyethyl, 2-cyanoethyl, methoxycarbonylmethyl, etc.; a substituted or unsubstituted aryl or hetaryl, aryloxy or hetaryloxy, arylthio or hetarylthio, arylsulfonyl or hetarylsulfonyl group having from about 2 to about 10 carbon atoms, such as phenyl, thienyl, pyridyl, imidazolyl, naphthyl, furyl, p-tolylsulfonyl, p-chlorophenylthio, m-(N-methyl sulfamoyl)phenoxy, etc.; a cycloalkyl group having from about 5 to about 7 carbon atoms, such as cyclohexyl, cyclopentyl, etc.; alkoxycarbonyl, such as ethoxycarbonyl or methoxycarbonyl; aryloxycarbonyl; acyl, such as acetyl or benzoyl; carbamoyl, such as N,N-dimethylcarbamoyl; a mono- or dialkylamino group, such as dimethylamino; a mono- or diarylamino group, such as morpholino, anilino or pyrrolidino; acylamido; sulfonamido; or sulfamoyl.

In a preferred embodiment of the invention,  $R^1$  is phenyl. In another preferred embodiment,  $R^2$  is dimethylamino or ethoxy. In yet another preferred embodiment,  $R^3$  is phenyl and  $R^4$  is phenyl or methyl. In yet another preferred embodiment,  $R^6$  is phenyl. In yet still another preferred embodiment,  $R^5$  is hydrogen.

Compounds included within the scope of the invention include the following:

Lum; a polycarbonate; poly(styrene-co-acrylonitrile), a poly(sulfone) or a poly(phenylene oxide). The binder may be used at a coverage of from about 0.1 to about 5 g/m<sup>2</sup>.

The dye layer of the dye-donor element may be coated on the support or printed thereon by a printing technique such as a gravure process.

Any material can be used as the support for the dye-donor element of the invention provided it is dimension-



| Cmpd. | $R^6$                                                        | $R^3$                                                                  | $R^4$                            | $R^1$                              | $R^2$                                                           | $R^5$                                         |
|-------|--------------------------------------------------------------|------------------------------------------------------------------------|----------------------------------|------------------------------------|-----------------------------------------------------------------|-----------------------------------------------|
| 1     | H                                                            | C <sub>6</sub> H <sub>5</sub>                                          | C <sub>6</sub> H <sub>5</sub>    | C <sub>6</sub> H <sub>5</sub>      | N(CH <sub>3</sub> ) <sub>2</sub>                                | H                                             |
| 2     | H                                                            | C <sub>6</sub> H <sub>5</sub>                                          | C <sub>6</sub> H <sub>5</sub>    | C <sub>6</sub> H <sub>5</sub>      | OC <sub>2</sub> H <sub>5</sub>                                  | H                                             |
| 3     | C <sub>6</sub> H <sub>5</sub>                                | C <sub>6</sub> H <sub>5</sub>                                          | CH <sub>3</sub>                  | C <sub>6</sub> H <sub>5</sub>      | N(CH <sub>3</sub> ) <sub>2</sub>                                | H                                             |
| 4     | C <sub>6</sub> H <sub>5</sub>                                | C <sub>6</sub> H <sub>5</sub>                                          | C <sub>2</sub> H <sub>5</sub>    | C <sub>6</sub> H <sub>5</sub>      | NHCH <sub>3</sub>                                               | H                                             |
| 5     | C <sub>6</sub> H <sub>5</sub>                                | C <sub>6</sub> H <sub>5</sub>                                          | C <sub>2</sub> H <sub>5</sub>    | C <sub>6</sub> H <sub>5</sub>      | NHC <sub>6</sub> H <sub>5</sub>                                 | H                                             |
| 6     | CH <sub>3</sub>                                              | C <sub>2</sub> H <sub>5</sub>                                          | C <sub>2</sub> H <sub>5</sub>    | C <sub>6</sub> H <sub>5</sub>      | NH <sub>2</sub>                                                 | CH <sub>3</sub>                               |
| 7     | S                                                            | n-C <sub>4</sub> H <sub>9</sub>                                        | H                                | CH <sub>3</sub>                    | N(CH <sub>3</sub> ) <sub>2</sub>                                | CN                                            |
|       |                                                              |                                                                        |                                  |                                    |                                                                 |                                               |
| 8     | p-CH <sub>3</sub> O <sub>C</sub> <sub>6</sub> H <sub>4</sub> | [—CH <sub>2</sub> ) <sub>2</sub> —O—(CH <sub>2</sub> ) <sub>2</sub> —] | C <sub>6</sub> H <sub>5</sub>    | C <sub>6</sub> H <sub>5</sub>      | OC <sub>6</sub> H <sub>5</sub>                                  | CN                                            |
| 9     | H                                                            | C <sub>6</sub> H <sub>5</sub>                                          | C <sub>6</sub> H <sub>5</sub>    | n-C <sub>4</sub> H <sub>9</sub>    | OC <sub>2</sub> H <sub>4</sub> OCH <sub>3</sub>                 | SCN                                           |
| 10    | S                                                            | C <sub>2</sub> H <sub>5</sub>                                          | C <sub>2</sub> H <sub>5</sub>    | C <sub>2</sub> H <sub>5</sub>      | N(C <sub>2</sub> H <sub>5</sub> )—C <sub>6</sub> H <sub>5</sub> | SO <sub>2</sub> —CH <sub>3</sub>              |
|       |                                                              |                                                                        |                                  |                                    |                                                                 |                                               |
| 11    | C <sub>2</sub> H <sub>5</sub> S—                             | i-C <sub>3</sub> H <sub>7</sub>                                        | H                                | H                                  |                                                                 | H                                             |
|       |                                                              |                                                                        |                                  |                                    |                                                                 |                                               |
| 12    | CH <sub>3</sub> CONH                                         | C <sub>2</sub> H <sub>5</sub>                                          | C <sub>2</sub> H <sub>5</sub>    | C <sub>6</sub> H <sub>5</sub>      | OCH <sub>2</sub> C <sub>6</sub> H <sub>5</sub>                  | COCH <sub>3</sub>                             |
| 13    | H                                                            | —C <sub>2</sub> H <sub>4</sub> O—COCH <sub>3</sub>                     | C <sub>2</sub> H <sub>5</sub>    | C <sub>5</sub> H <sub>4</sub> N    | N(CH <sub>3</sub> ) <sub>2</sub>                                | Cl                                            |
| 14    | SCN                                                          | —C <sub>2</sub> H <sub>4</sub> OH                                      | C <sub>2</sub> H <sub>5</sub>    | C <sub>5</sub> H <sub>5</sub>      | OCH <sub>3</sub>                                                | H                                             |
| 15    | C <sub>6</sub> H <sub>5</sub>                                | —CH <sub>2</sub> CF <sub>3</sub>                                       | —CH <sub>2</sub> CF <sub>3</sub> | CH <sub>3</sub>                    | N(CH <sub>3</sub> ) <sub>2</sub>                                | CN                                            |
| 16    | C <sub>2</sub> H <sub>5</sub> O—                             | CH <sub>3</sub>                                                        | CH <sub>3</sub>                  | p-Cl—C <sub>6</sub> H <sub>4</sub> | NHC <sub>2</sub> H <sub>5</sub>                                 | CO <sub>2</sub> C <sub>2</sub> H <sub>5</sub> |
| 17    | Cl                                                           | i-C <sub>3</sub> H <sub>7</sub>                                        | H                                | C <sub>6</sub> H <sub>5</sub>      | N(CH <sub>3</sub> ) <sub>2</sub>                                | H                                             |
| 18    | CH <sub>3</sub> SO <sub>2</sub>                              | C <sub>2</sub> H <sub>5</sub>                                          | C <sub>2</sub> H <sub>5</sub>    | C <sub>2</sub> H <sub>5</sub>      | OC <sub>2</sub> H <sub>5</sub>                                  | N(CH <sub>3</sub> ) <sub>2</sub>              |
| 19    | C <sub>6</sub> H <sub>5</sub>                                | C <sub>2</sub> H <sub>4</sub> CN                                       | C <sub>2</sub> H <sub>4</sub> CN | C <sub>6</sub> H <sub>5</sub>      | OCH <sub>3</sub>                                                | H                                             |
| 20    | CH <sub>3</sub>                                              | —CH <sub>2</sub> C <sub>6</sub> H <sub>5</sub>                         | C <sub>2</sub> H <sub>5</sub>    | C <sub>6</sub> H <sub>5</sub>      | N(CH <sub>3</sub> )—(C <sub>2</sub> H <sub>5</sub> )            | CN                                            |

These dyes may be prepared analogous to the method described in Weaver et al. U.S. Pat. No. 3,247,211, and the synthesis of the requisite aminothiazole aldehydes is described in J. Chem. Soc., Perkins Trans I, 341-7 (1983), the disclosures of which are hereby incorporated by reference.

A dye-barrier layer may be employed in the dye-donor elements of the invention to improve the density of the transferred dye. Such dye-barrier layer materials include hydrophilic materials such as those described and claimed in U.S. Pat. No. 4,716,144 by Vanier, Lum and Bowman.

The dye in the dye-donor element of the invention is dispersed in a polymeric binder such as a cellulose derivative, e.g., cellulose acetate hydrogen phthalate, cellulose acetate, cellulose acetate propionate, cellulose acetate butyrate, cellulose triacetate or any of the materials described in U.S. Pat. No. 4,700,207 of Vanier and

ally stable and can withstand the heat of the thermal printing heads. Such materials include polyesters such as poly(ethylene terephthalate); polyamides; polycarbonates; glassine paper; condenser paper; cellulose esters such as cellulose acetate; fluorine polymers such as polyvinylidene fluoride or poly(tetrafluoroethylene-co-hexafluoropropylene); polyethers such as polyoxymethylene; polyacetals; polyolefins such as polystyrene, polyethylene, polypropylene or methylpentane polymers; and polyimides such as polyimide-amides and polyetherimides. The support generally has a thickness of from about 2 to about 30  $\mu$ m. It may also be coated with a subbing layer, if desired, such as those materials described in U.S. Pat. No. 4,695,288 of Ducharme or U.S. application Ser. No. 079,613 of Henzel, filed July 30, 1987.

The reverse side of the dye-donor element may be coated with a slipping layer to prevent the printing head from sticking to the dye-donor element. Such a slipping layer would comprise a lubricating material such as a surface active agent, a liquid lubricant, a solid lubricant or mixtures thereof, with or without a polymeric binder. Preferred lubricating materials include oils or semi-crystalline organic solids that melt below 100° C. such as poly(vinyl stearate), beeswax, perfluorinated alkyl ester polyethers, poly(caprolactone), silicone oil, poly(tetrafluoroethylene), carbowax, poly(ethylene glycols), or any of those materials disclosed in U.S. application Ser. Nos. 925,949 of Vanier, Harrison and Kan, filed Nov. 3, 1986; 925,948 of Harrison, Vanier and Kan, filed Nov. 3, 1986; 076,433 of Henzel, Lum and Vanier, filed July 21, 1987, and 062,796 of Vanier and Evans, filed June 16, 1987. Suitable polymeric binders for the slipping layer include poly(vinyl alcohol-co-butyral), poly(vinyl alcohol-co-acetal), poly(styrene), poly(vinyl acetate), cellulose acetate butyrate, cellulose acetate propionate, cellulose acetate or ethyl cellulose.

The amount of the lubricating material to be used in the slipping layer depends largely on the type of lubricating material, but is generally in the range of about 0.001 to about 2 g/m<sup>2</sup>. If a polymeric binder is employed, the lubricating material is present in the range of 0.1 to 50 weight %, preferably 0.5 to 40, of the polymeric binder employed.

The dye-receiving element that is used with the dye-donor element of the invention usually comprises a support having thereon a dye image-receiving layer. The support may be a transparent film such as a poly(ether sulfone), a polyimide, a cellulose ester such as cellulose acetate, a poly(vinyl alcohol-co-acetal) or a poly(ethylene terephthalate). The support for the dye-receiving element may also be reflective such as baryta-coated paper, polyethylene-coated paper, white polyester (polyester with white pigment incorporated therein), an ivory paper, a condenser paper or a synthetic paper such as duPont Tyvek®.

The dye image-receiving layer may comprise, for example, a polycarbonate, a polyurethane, a polyester, polyvinyl chloride, poly(styrene-co-acrylonitrile), poly(caprolactone) or mixtures thereof. The dye image-receiving layer may be present in any amount which is effective for the intended purpose. In general, good results have been obtained at a concentration of from about 1 to about 5 g/m<sup>2</sup>.

As noted above, the dye-donor elements of the invention are used to form a dye transfer image. Such a process comprises imagewise-heating a dye-donor element as described above and transferring a dye image to a dye-receiving element to form the dye transfer image.

The dye-donor element of the invention may be used in sheet form or in a continuous roll or ribbon. If a continuous roll or ribbon is employed, it may have only the dye thereon as described above or may have alternating areas of other different dyes, such as sublimable cyan and/or magenta and/or yellow and/or black or other dyes. Such dyes are disclosed in U.S. Pat. Nos. 4,541,830; 4,698,651 of Moore, Weaver and Lum; 4,695,287 of Evans and Lum; and 4,701,439 of Weaver, Moore and Lum; and U.S. application Ser. Nos. 059,442 of Byers and Chapman, filed June 8, 1987; 059,443 of Evans and Weber, filed June 8, 1987; 095,796 of Evans and Weber, filed Sept. 14, 1987; and 123,441 of Byers, Chapman and McManus, filed Nov. 20, 1987, the disclosures of which are hereby incorporated by reference.

Thus, one-, two-, three- or four-color elements (or higher numbers also) are included within the scope of the invention.

In a preferred embodiment of the invention, the dye-donor element comprises a poly(ethylene terephthalate) support coated with sequential repeating areas of magenta, cyan and a dye as described above which is of yellow hue, and the above process steps are sequentially performed for each color to obtain a three-color dye transfer image. Of course, when the process is only performed for a single color, then a monochrome dye transfer image is obtained.

Thermal printing heads which can be used to transfer dye from the dye-donor elements of the invention are available commercially. There can be employed, for example, a Fujitsu Thermal Head (FTP-040 MSC001), a TDK Thermal Head F415 HH7-1089 or a Rohm Thermal Head KE 2008-F3.

A thermal dye transfer assemblage of the invention comprises

(a) a dye-donor element as described above, and  
(b) a dye-receiving element as described above, the dye-receiving element being in a superposed relationship with the dye-donor element so that the dye layer of the donor element is in contact with the dye image-receiving layer of the receiving element.

The above assemblage comprising these two elements may be preassembled as an integral unit when a monochrome image is to be obtained. This may be done by temporarily adhering the two elements together at their margins. After transfer, the dye-receiving element is then peeled apart to reveal the dye transfer image.

When a three-color image is to be obtained, the above assemblage is formed on three occasions during the time when heat is applied by the thermal printing head. After the first dye is transferred, the elements are peeled apart. A second dye-donor element (or another area of the donor element with a different dye area) is then brought in register with the dye-receiving element and the process repeated. The third color is obtained in the same manner.

The following example is provided to illustrate the invention.

#### EXAMPLE

A yellow dye-donor element was prepared by coating the following layers in the order recited on a 6 μm poly(ethylene terephthalate) support:

- (1) Subbing layer of duPont Tyzor TBT® titanium tetra-n-butoxide (0.16 g/m<sup>2</sup>) coated from a n-butyl alcohol and n-propyl acetate solvent mixture, and
- (2) Dye layer containing dye 1 identified above of yellow hue (0.47 mmoles/m<sup>2</sup>), FC-431® surfactant (3M Corp.) (0.002 g/m<sup>2</sup>), in a cellulose acetate-propionate (2.5% acetyl, 48% propionyl) binder (weight equal to 2.0X that of the dye) coated from a cyclopentanone, toluene, and methanol solvent mixture.

A slipping layer was coated on the back side of the element similar to that disclosed in U.S. application Ser. No. 184,316 of Vanier et al, filed Apr. 21, 1988.

A dye-receiving element was prepared by coating a solution of Makrolon 5705® (Bayer AG Corporation) polycarbonate resin (2.9 g/m<sup>2</sup>) and polycaprolactone (0.8 g/m<sup>2</sup>) in methylene chloride on a pigmented polyethylene-overcoated paper stock.

The dye side of the dye-donor element strip approximately 10 cm × 13 cm in area was placed in contact with

the dye image-receiving layer of the dye-receiver element of the same area. The assemblage was clamped to a stepper-motor driven 60 mm diameter rubber roller and a TDK Thermal Head (No. L-231) (thermostatted at 26° C.) was pressed with a force of 8.0 pounds (3.6 kg) against the dye-donor element side of the assemblage pushing it against the rubber roller.

The imaging electronics were activated causing the donor/receiver assemblage to be drawn between the printing head and roller at 6.9 mm/sec. Coincidentally, the resistive elements in the thermal print head were pulsed at 29  $\mu$ sec/pulse at 128  $\mu$ sec intervals during the 33 msec/dot printing time. A stepped density image was generated by incrementally increasing the number of pulses/dot from 0 to 255. The voltage supplied to the print head was approximately 23.5 volts, resulting in an instantaneous peak power of 1.3 watts/dot and a maximum total energy of 9.6 mJoules/dot.

The dye-receiving element was separated from the dye-donor element. The status A blue reflection densities of each stepped image consisting of a series of 11 graduated density steps 1 cm  $\times$  1 cm were read.

The images were then subjected to High-Intensity Daylight fading (HID-fading) for 7 days, 50 kLux, 5400° K., 32° C., approximately 25% RH and the densities were reread. The percent density loss was calculated from D-max (the highest density step). The  $\lambda$ -max of each dye in an acetone solution was also determined. The following results were obtained:

TABLE 3

| Dye-Donor Element w/ Compound | Fade Test (days) | $\lambda$ -max | Status A Blue Density | % Loss After Fade |
|-------------------------------|------------------|----------------|-----------------------|-------------------|
| 1                             | 7                | 437 nm         | 2.1                   | 6                 |
| 2                             | 7                | 431 nm         | 2.1                   | 3                 |
| 3                             | 7                | 454 nm         | 1.8                   | 5                 |
| Control 1                     | 7                | 426 nm         | 1.8                   | 86                |
| Control 2                     | 7                | 436 nm         | 2.2                   | 50                |
| Control 3                     | 7                | 447 nm         | 2.4                   | 22                |
| Control 4                     | 7                | 439 nm         | 2.3                   | 21                |

The above results indicate that the yellow dyes according to the invention have improved light stability in comparison to several prior art control yellow dyes.

45  
50

-continued

## Control Compounds



## Control Compound 4



The invention has been described in detail with particular reference to preferred embodiments thereof, but it will be understood that variations and modifications can be effected within the spirit and scope of the invention.

What is claimed is:

1. A dye-donor element for thermal dye transfer comprising a support having thereon a dye dispersed in a polymeric binder, said dye comprising a 2-aminothiazol-5-ylmethylene-2-pyrazoline-5-one, said pyrazoline ring being substituted in the 3-position by an amino group or an alkoxy group.

2. The element of claim 1 wherein said dye has the formula:



wherein R<sup>1</sup> represents hydrogen, a substituted or unsubstituted alkyl group having from 1 to about 10 carbon atoms, a cycloalkyl group having from about 5 to about 7 carbon atoms, or a substituted or unsubstituted aryl or hetaryl group having from about 2 to about 10 carbon atoms;

R<sup>2</sup> represents an alkoxy group having from 1 to about 10 carbon atoms or a primary, secondary or tertiary amino group;

R<sup>3</sup> and R<sup>4</sup> each represents R<sup>1</sup>, with the proviso that only one of R<sup>3</sup> and R<sup>4</sup> may be hydrogen, or R<sup>3</sup> and R<sup>4</sup> can be joined together to form, along with the nitrogen to which they are attached, a 5- or 6-membered heterocyclic ring;

R<sup>5</sup> and R<sup>6</sup> each independently represents hydrogen; halogen; cyano; thiocyanato; a substituted or unsubstituted alkyl, alkoxy, alkylthio or alkylsulfonyl group having from 1 to about 10 carbon atoms; a substituted or unsubstituted aryl or hetaryl, aryloxy or hetaryloxy, arylthio or hetarylthio, arylsulfonyl or hetaryl sulfonyl group having from about 2 to about 10 carbon atoms; a cycloalkyl group having from about 5 to about 7 carbon atoms; alkoxy carbonyl;

40

## Control Compounds

## Control Compound 1



## Control Compound 2



## Control Compound 3

bonyl; aryloxycarbonyl; acyl; carbamoyl; mono- or dialkylamino; mono- or diarylamino; acylamido; sulfonamido; or sulfamoyl.  
 3. The element of claim 2 wherein R<sup>1</sup> is phenyl and R<sup>2</sup> is dimethylamine or ethoxy.

4. The element of claim 2 wherein R<sup>3</sup> is phenyl and R<sup>4</sup> is phenyl or methyl.

5. The element of claim 2 wherein R<sup>6</sup> is phenyl.

6. The element of claim 2 wherein R<sup>5</sup> is hydrogen.

7. The element of claim 1 wherein said support comprises poly(ethylene terephthalate) and the side of the support opposite the side having thereon said dye layer is coated with a slipping layer comprising a lubricating material.

8. The element of claim 1 wherein said dye layer comprises sequential repeating areas of magenta, cyan and said dye which is of yellow hue.

9. In a process of forming a dye transfer image comprising imagewise-heating a dye-donor element comprising a support having thereon a dye layer comprising a dye dispersed in a polymeric binder and transferring a dye image to a dye-receiving element to form said dye transfer image, the improvement wherein said dye comprises a 2-amino-thiazol-5-ylmethylene-2-pyrazoline-5-one, said pyrazoline ring being substituted in the 3-position by an amino group or an alkoxy group.

10. The process of claim 9 wherein said dye has the formula:



wherein R<sup>1</sup> represents hydrogen, a substituted or unsubstituted alkyl group having from 1 to about 40 10 carbon atoms, a cycloalkyl group having from about 5 to about 7 carbon atoms, or a substituted or unsubstituted aryl or hetaryl group having from about 2 to about 10 carbon atoms;

R<sup>2</sup> represents an alkoxy group having from 1 to about 45 10 carbon atoms or a primary, secondary or tertiary amino group;

R<sup>3</sup> and R<sup>4</sup> each represents R<sup>1</sup>, with the proviso that only one of R<sup>3</sup> and R<sup>4</sup> may be hydrogen, or R<sup>3</sup> and R<sup>4</sup> can be joined together to form, along with the nitrogen to which they are attached, a 5- or 6-membered heterocyclic ring;

R<sup>5</sup> and R<sup>6</sup> each independently represents hydrogen; halogen; cyano; thiocyanato; a substituted or unsubstituted alkyl, alkoxy, alkylthio or alkylsulfonyl group having from 1 to about 10 carbon atoms; a substituted or unsubstituted aryl or hetaryl, aryloxy or hetaryloxy, arylthio or hetarylthio, arylsulfonyl or hetaryl sulfonyl group having from about 2 to 60 about 10 carbon atoms; a cycloalkyl group having from about 5 to about 7 carbon atoms; alkoxy carbonyl; aryloxycarbonyl; acyl; carbamoyl; mono- or dialkylamino; mono- or diarylamino; acylamido; sulfonamido; or sulfamoyl.

11. The process of claim 10 wherein R<sup>1</sup> is phenyl and R<sup>2</sup> is dimethylamine or ethoxy.

12. The process of claim 10 wherein R<sup>3</sup> is phenyl and R<sup>4</sup> is phenyl or methyl.

13. The process of claim 10 wherein R<sup>6</sup> is phenyl.

14. The process of claim 10 wherein R<sup>5</sup> is hydrogen.

5 15. The process of claim 9 wherein said support is poly(ethylene terephthalate) which is coated with sequential repeating areas of magenta, cyan and said dye which is of yellow hue, and said process steps are sequentially performed for each color to obtain a three-color dye transfer image.

10 16. In a thermal dye transfer assemblage comprising:

(a) a dye-donor element comprising a support having thereon a dye layer comprising a dye dispersed in a polymeric binder, and

15 (b) a dye-receiving element comprising a support having thereon a dye image-receiving layer, said dye-receiving element being in a superposed relationship with said dye-donor element so that said dye layer is in contact with said dye image-receiving layer, the improvement wherein said dye comprises a 2-amino-thiazol-5-ylmethylene-2-pyrazoline-5-one, said pyrazoline ring being substituted in the 3-position by an amino group or an alkoxy group.

20 25 17. The assemblage of claim 16 wherein said dye has the formula:



30 35 wherein R<sup>1</sup> represents hydrogen, a substituted or unsubstituted alkyl group having from 1 to about 10 carbon atoms, a cycloalkyl group having from about 5 to about 7 carbon atoms, or a substituted or unsubstituted aryl or hetaryl group having from about 2 to about 10 carbon atoms;

R<sup>2</sup> represents an alkoxy group having from 1 to about 10 carbon atoms or a primary, secondary or tertiary amino group;

R<sup>3</sup> and R<sup>4</sup> each represents R<sup>1</sup>, with the proviso that only one of R<sup>3</sup> and R<sup>4</sup> may be hydrogen, or R<sup>3</sup> and R<sup>4</sup> can be joined together to form, along with the nitrogen to which they are attached, a 5- or 6-membered heterocyclic ring;

R<sup>5</sup> and R<sup>6</sup> each independently represents hydrogen; halogen; cyano; thiocyanato; a substituted or unsubstituted alkyl, alkoxy, alkylthio or alkylsulfonyl group having from 1 to about 10 carbon atoms; a substituted or unsubstituted aryl or hetaryl, aryloxy or hetaryloxy, arylthio or hetarylthio, arylsulfonyl or hetaryl sulfonyl group having from about 2 to about 10 carbon atoms; a cycloalkyl group having from about 5 to about 7 carbon atoms; alkoxy carbonyl; aryloxycarbonyl; acyl; carbamoyl; mono- or dialkylamino; mono- or diarylamino; acylamido; sulfonamido; or sulfamoyl.

18. The assemblage of claim 17 wherein R<sup>1</sup> is phenyl and R<sup>2</sup> is dimethylamine or ethoxy.

19. The assemblage of claim 17 wherein R<sup>3</sup> is phenyl and R<sup>4</sup> is phenyl or methyl.

65 20. The assemblage of claim 17 wherein R<sup>6</sup> is phenyl and R<sup>5</sup> is hydrogen.

\* \* \* \* \*